

Patented July 23, 1929.

1,721,702

# UNITED STATES PATENT OFFICE.

ARMAN E. BECKER, OF ELIZABETH, NEW JERSEY, ASSIGNOR TO STANDARD OIL DEVELOPMENT COMPANY, A CORPORATION OF DELAWARE.

## BELT DRESSING AND PROCESS OF MAKING THE SAME.

No Drawing.

Application filed June 25, 1925. Serial No. 39,611.

This invention relates to improvements in oleaginous compositions for the treatment of leather and the like. The principal object of the invention is to provide a leather belt dressing characterized by high penetrating power, stability in the presence of moisture and under varying atmospheric conditions, substantial freedom from stickiness and drying tendencies, and other advantageous properties.

10 In accordance with a preferred form of my invention, a mixture of the following ingredients in about the proportions stated is prepared:

| 16 Lubricating oil (100-300 seconds Saybolt at 100° F.) | Per cent. |
|---------------------------------------------------------|-----------|
| Oil soluble sodium sulfonate                            | 20        |
| Neat's-foot oil                                         | 10        |

Any suitable mineral oil may be used, preferably of the lubricating type and within the viscosity range stated.

The oil-soluble sodium sulfonate may be prepared in the well-known manner by alcohol extraction of oil which has been acid treated and neutralized for the production of white oils and the like. This sodium sulfonate frequently contains a small amount of residual alkali, usually less than 2%. When this is the case, rosin may be added in amount sufficient only to neutralize residual alkali. The rosin is converted into a soap and does not have the objectionable properties which rosin is sometimes said to have in prior belt dressings in which it has been present as such.

35 Other organic neutralizing compounds, such as animal or vegetable oils, saponifiable by alkali in the presence of oil, may be used. When sulfonic soaps free from caustic are available the rosin or the like may be omitted.

40 It is feasible to neutralize excess caustic before incorporating the sulfonate in the oil, but the procedure described is generally more convenient.

45 The following ingredients may be compounded when a typical alkali-containing sulfonate is used:

| 50 Lubricating oil (100-300 seconds Saybolt at 100° F.) | Per cent. |
|---------------------------------------------------------|-----------|
| Oil soluble sodium sulfonate                            | 20        |
| Rosin                                                   | 2.6       |
| Neat's-foot oil                                         | 7.4       |

While I prefer to use a small amount of

neat's-foot oil, it is not a necessary ingredient of my composition. The improved belt dressing is made up by dissolving the sodium sulfonate in the mineral oil. Heating and stirring may be necessary to secure quick solution of the sulfonate. When there is residual alkali to be neutralized, rosin or the like is added and the mixture is heated and stirred. The oil is next allowed to cool and settle, during which some insoluble impurities may settle out. The neat's-foot oil, if this oil is to be used, is added while the oil is still warm.

The preferred proportions given may be varied widely, for example I may use as much as 50% of sodium sulfonate, the remainder of the composition consisting of lubricating oil. Although higher percentages of sodium sulfonate may be used, ordinarily no advantage is derived from so doing. Less than 10% of sodium sulfonate will not in general give the desired result. Other alkali metal sulfonates may be substituted for sodium sulfonate.

Tests of my belt dressing show that it renders the leather very pliable, probably due to its unusual penetrating power. The leather is soft and adheres well to the pulley. The dressing does not make the leather objectionably sticky or adherent to the driven surface. Water which may come in contact with the surface of the leather has no substantial adverse effect on the dressing. Leather treated with the dressing will absorb a reasonable amount of lubricating oil which may happen to come in contact with it from near by bearings, and the annoyance of a slippery belt is therefore generally avoided.

I claim:

1. A composition adapted for use as a belt dressing, or the like, comprising a mineral oil of lubricating grade, oil-soluble sodium sulfonate, and neat's-foot oil.

2. A composition adapted for use as a belt dressing, or the like, comprising a mineral oil of lubricating grade, oil-soluble sodium sulfonate, saponified rosin, and neat's-foot oil.

3. A composition adapted for use as a belt dressing, or the like, comprising about 70% by weight of a mineral lubricating oil, about 20% of oil-soluble sodium sulfonate, about 2.6% of saponified rosin, and about 7.4% of neat's-foot oil.

4. Process of making a composition adapted for use as a belt dressing, or the like, com-

prising mixing a mineral oil of lubricating grade and an oil-soluble sulfonate containing grade and an oil-soluble sulfonate containing free alkali, adding rosin to react with such alkali, heating and stirring the mixture to 10 alkali, heating and stirring the mixture to facilitate neutralization, cooling, settling, and removing any deposited impurities.

5. Process of making a composition adapted for use as a belt dressing, or the like, comprising mixing a mineral oil of lubricating

ARMAN E. BECKER.